# EUROPEAN PATENT SPECIFICATION

(11) **EP 1 522 648 B1**
(45) Date of publication and mention of the grant of the patent: **14.02.2007**
(21) Application number: 04104942.0
(22) Date of filing: 08.10.2004
(51) Int. Cl.: E04C 2/34, E04C 2/24

(54) **Flat wall panel at least substantially made of cellulose material**
Flaches Wandelement aus Zellulose
Elément de paroi plat en cellulose

(30) Priority: 10.10.2003 NL 1024505
(43) Date of publication of application: 13.04.2005
(73) Proprietor: Unda Maris B.V., 1689 AN Zwaag (NL)
(72) Inventor: Snel, Wilhelmus Jan Reinier Karel, 1689 AN, Zwaag (NL)
(74) Representative: Hooiveld, Arjen Jan Winfried

(56) References cited:
- EP-A- 1 180 564
- GB-A- 600 607
- GB-A- 1 100 951
- GB-A- 1 542 730
- US-A- 3 542 636
- US-A- 4 351 870

## Description

The invention relates to a flat wall panel at least substantially made of cellulose material, wherein the wall panel is at least substantially made of layers of paper/cardboard, each layer at least substantially being made up of a corrugated sublayer and a flat sublayer provided on one side thereof, which layers of paper/cardboard are interconnected via an adhesive, wherein the wall panel is impregnated, and wherein at least one strengthening layer having a greater elasticity modulus than the layers of paper/cardboard is provided, which strengthening layer is connected to a layer of paper/cardboard on one side of the wall panel via an adhesive. The invention also relates to a method for manufacturing said wall panel.

Such a wall panel is known from British patent publication no. 1,542,730 (Tri-Wall Containers Ltd). In this prior art document a flame resistant, fire retardant material is mentioned, particularly containing a borax or an ammonium based compound, said material being applied through a dipping process. A disadvantage of this known wall panel is that in practice it suffers from a lack of constructional stiffness, which severely limits its practical use.
The object of the invention is to improve the wall panel that is known from the aforesaid British patent publication, in the sense that a wall panel having an optimum constructional stiffness is provided for use as a construction element of a building, as a wall panel in, for example, a separation wall, etc. It is noted that the term wall panel is understood to include an element for use in a wall, a floor, a ceiling, a roof, etc.

According to the invention, a wall panel of the kind referred to in the introduction is characterized in that the wall panel is impregnated with a resinous material, and that the wall panel is at least substantially made of an even number of layers of paper/cardboard, wherein the wall panel is mirror symmetrical with respect to a central longitudinal plane of the wall panel, said at least one strengthening layer having an elasticity modulus greater than or equal to 50 GPA.

In other words, a plate-shaped material is provided which is hardly deformable, if at all, wherein "warping" is prevented at all times. Experiments have shown that the present construction leads to an unexpectedly great constructional stiffness of the wall panel, so that it is possible to subject the wall panel to large forces without the dimensional stability being affected. The constructional stiffness is increased even further by using a strengthening layer having an elasticity modulus greater than or equal to 100 GPA, in particular greater than or equal to 150 GPA, more in particular greater than or equal to 200 GPA, more in particular greater than or equal to 300 GPA, more in particular greater than or equal to 400 GPA.

The aforesaid resinous material with which the wall panel according to the invention is impregnated, is preferably an epoxy resin, a polyurethane resin, a polyester resin or a phenol resin. Fire-resistant and/or fire-retarding agents may be added thereto. Preferably, the resinous material with which the wall panel according to the invention is impregnated also functions as an adhesive for adhering two layers of paper/cardboard together, so that a separate adhesive, such as a glue, is not required. To that end, sets consisting of a corrugated sublayer and a flat sublayer provided on one side thereof, which sublayers are already impregnated with the resinous material, can be placed on top of each other so as to be adhered together (after the resinous material has dried).

In a preferred embodiment of a wall panel according to the invention, the wall panel comprises two strengthening layers, which are connected to a layer of paper/cardboard on either side of the wall panel via an adhesive. Thus a sandwich construction is obtained, in which the whole of various adhered-together layers of paper/cardboard is connected to a less elastic strengthening layer on both flat outer sides. The result is an even greater constructional stiffness having a corresponding dimensional stability.

It is noted that impregnating the wall panel with, for example, a resinous material not only has the advantage of providing a greater constructional stiffness, but also of providing protection against external influences, such as moisture. As a result of said additional stiffness, fewer layers of corrugated paper/cardboard are in principle needed in order to give the flat panel the required stiffness. Said impregnation preferably takes place by means of vapour deposition, spraying or otherwise, said vapour deposition or spraying taking place in a direction parallel to the direction of the "cell structure" of the corrugated paper/cardboard that is used. Said impregnation may also be effected with mechanical means, wherein toothed and/or flat rollers are used for pressing the impregnating medium into the paper/cardboard.

In another preferred embodiment of a wall panel according to the invention, the strengthening layer comprise a fibre material. In particular, the fibre material consists of glass fibres, carbon fibres, mineral fibres and/or synthetic fibres. Said synthetic fibres may e.g. be fibres of the type known under the brand names "Kevlar" or "Twaron".

In another preferred embodiment of a plate-shaped material according to the invention, the strengthening layer comprises a layer of a plastic material. The plastic of said layer of plastic material is preferably selected from the group consisting of PVC-U, PP, PE, ABS, PVC-C and PVDF. It is noted that the above abbreviations relate to the following (plastic) materials.
- PVC-U: Polyvinyl chloride (without plasticizer)
- PP: Polypropylene
- PE: Polyethylene
- ABS: Acrylonitrile-Butadiene-Styrene
- PVC-C: Polyvinyl chloride (post-chlorinated)
- PVDF: Polyvinylydene fluoride

In another preferred embodiment of wall panel according to the invention, the strengthening layer comprises a layer of rubber. The rubber of said layer of rubber is preferably selected from the group consisting of EPDM or NBR. In another preferred variant, the strengthening layer is made of a metal, in particular stainless steel, or wood.

As already said before, the invention also relates to a method for manufacturing a wall panel according to the invention wherein the wall panel is at least substantially made of an even number of layers of paper/cardboard, each layer at least substantially being made up of a corrugated sublayer and a flat sublayer provided on one side thereof, which layers of paper/cardboard are interconnected via an adhesive applied to the corrugations of the corrugated sublayers, wherein the wall panel is impregnated, with a resinous material, wherein at least one strengthening layer having a greater elasticity modulus than the layers of paper/cardboard is provided, which strengthening layer is connected to a layer of paper/cardboard on one side of the wall panel via an adhesive, and wherein the wall panel is mirror symmetrical with respect to a central longitudinal plane of the wall panel, said at least one strengthening layer having an elasticity modulus greater than or equal to 50 GPA.

It is noted that the term paper is usually used for lighter types of paper; in the case of a heavier quality, the term cardboard is frequently used. Within the framework of the invention, the terms paper, cardboard and weight are not intended to be limitative as regards the type of material to be used.

The invention will now be explained in more detail with reference to figures illustrated in a drawing of a preferred variant of the invention, in which Fig. 1 is a schematic, perspective view of the present wall panel, Fig. 2 is a detail view of Fig. 1, and Fig. 3 is an exploded view of the wall panel of Fig. 1.

The figure shows a flat wall panel 1 according to the invention in the form of a sandwich", in the sense that a core 2 built up of several layers of corrugated cardboard is connected on either side to a less elastic strengthening layer 3 of a thin material having an elasticity modulus of about 400 Gpa.

In this case, four layers of corrugated cardboard are provided, which are each built up of corrugated sublayer 4 and a flat sublayer 5 glued to one side thereof, using a glue applied to the corrugations 6 of the corrugated sublayer 4. The core 2 is impregnated with a resinous material. As already said before, the strengthening layers 3 are glued to both sides of the core 2.

The wall panel 1 is mirror symmetrical with respect to a central longitudinal plane 7 of the wall panel 1.

It is noted that the invention is not limited to the embodiment as shown in the figures, but that it also extends to other variants that fall within the scope of the appended claims. Thus it will be apparent to those skilled in the art that the wall panel may exhibit a (slight) curvature, whilst the wall panel may also comprise a curved longitudinal edge.

## Claims

1. A flat wall panel (1) at least substantially made of cellulose material, wherein the wall panel (1) is at least substantially made of layers of paper/cardboard, each layer (4) at least substantially being made up of a corrugated sublayer (5) and a flat sublayer provided on one side thereof, which layers of paper/cardboard are interconnected via an adhesive, wherein the wall panel (1) is impregnated, and wherein at least one strengthening layer (3) having a greater elasticity modulus than the layers of paper/cardboard is provided, which strengthening layer (3) is connected to a layer of paper/cardboard on one side of the wall panel (1) via an adhesive, **characterized in that** the wall panel (1) is impregnated with a resinous material, and that the wall panel (1) is at least substantially made of an even number of layers of paper/cardboard, wherein the wall panel (1) is mirror symmetrical with respect to a central longitudinal plane (7) of the wall panel (1), said at least one strengthening layer (3) having an elasticity modulus greater than or equal to 50 GPA.

2. A wall panel (1) according to claim 1, wherein two strengthening layers (3) are provided, which are connected to a layer of paper/cardboard on either side of the wall panel (1) via an adhesive.

3. A wall panel (1) according to claim 1 or 2, wherein the strengthening layer(s) (3) comprise(s) a fibre material.

4. A wall panel (1) according to claim 3, wherein the fibre material consists of glass fibres, carbon fibres, mineral fibres and/or synthetic fibres.

5. A wall panel (1) according to any one of the preceding claims 1-4, wherein the strengthening layer(s) (3) comprise(s) a layer of plastic material.

6. A wall panel (1) according to any one of the preceding claims 1-5, wherein the strengthening layer(s) (3) comprise(s) a layer of rubber.

7. A wall panel (1) according to any one of the preceding claims 1-6, wherein the strengthening layer(s) (3) is (are) made of a metal.

8. A wall panel (1) according to any one of the preceding claims 1-7, wherein the strengthening layer(s) (3) is (are) made of wood.

9. A method for manufacturing a flat wall panel (1) according to any one of the preceding claims 1-8, **characterized in that** the wall panel (1) is at least substantially made of an even number of layers of paper/cardboard, each layer at least substantially being made up of a corrugated sublayer (4) and a flat sublayer (5) provided on one side thereof, which layers of paper/cardboard are interconnected via an adhesive applied to the corrugations (6) of the corrugated sublayers (4), wherein the wall panel (1) is impregnated, with a resinous material, wherein at least one strengthening layer (3) having a greater elasticity modulus than the layers of paper/cardboard is provided, which strengthening layer (3) is connected to a layer of paper/cardboard on one side of the wall panel (1) via an adhesive, and wherein the wall panel (1) is mirror symmetrical with respect to a central longitudinal plane (7) of the wall panel (1), said at least one strengthening layer (3) having an elasticity modulus greater than or equal to 50 GPA.

## Patentansprüche

1. Flaches Wandelement (1), das wenigstens im wesentlichen aus Zellulosematerial hergestellt ist, wobei das Wandelement (1) wenigstens im wesentlichen hergestellt ist aus Schichten aus Papier/Pappe, wobei jede Schicht (4) wenigstens im wesentlichen gebildet ist aus einer gewellten Unterschicht (5) und einer ebenen Unterschicht, die auf einer Seite derselben bereitgestellt ist, welche Schichten aus Papier/Pappe miteinander über einen Klebstoff verbunden sind, wobei das Wandelement (1) imprägniert ist, und wobei wenigstens eine Verstärkungsschicht (3) mit einem größeren Elastizitätsmodul als die Schichten aus Papier/Pappe bereitgestellt ist, welche Verstärkungsschicht (3) mit einer Schicht aus Papier/Pappe auf einer Seite des Wandelements (1) über einen Klebstoff verbunden ist, **dadurch gekennzeichnet, daß** das Wandelement (1) mit einem harzartigen Material imprägniert ist, und daß das Wandelement (1) wenigstens im wesentlichen hergestellt ist aus einer geraden Anzahl von Schichten aus Papier/Pappe, wobei das Wandelement (1) spiegelsymmetrisch ist in Bezug auf eine zentrale Längsebene (7) des Wandelements (1), wobei die wenigstens eine Verstärkungsschicht (3) einen Elastizitätsmodul von größer als oder gleich 50 GPA aufweist.

2. Wandelement (1) nach Anspruch 1, wobei zwei Verstärkungsschichten (3) vorgesehen sind, die an einer Schicht aus Papier/Pappe auf jeder Seite des Wandelements (1) über einen Klebstoff gebunden sind.

3. Wandelement (1) nach Anspruch 1 oder 2, wobei die Verstärkungsschicht(en) (3) ein Fasermaterial umfaßt bzw. umfassen.

4. Wandelement (1) nach Anspruch 3, wobei das Fasermaterial aus Glasfasern, Kohlefasern, Mineralfasern und/oder synthetischen Fasern besteht.

5. Wandelement (1) nach einem der vorangehenden Ansprüche 1 bis 4, wobei die Verstärkungsschicht(en) (3) eine Schicht aus Kunststoffmaterial umfaßt bzw. umfassen.

6. Wandelement (1) nach einem der vorangehenden Ansprüche 1 bis 5, wobei die Verstärkungsschicht(en) (3) eine Kautschukschicht umfaßt bzw. umfassen.

7. Wandelement (1) nach einem der vorangehenden Ansprüche 1 bis 6, wobei die Verstärkungsschicht(en) (3) aus einem Metall hergestellt ist bzw. sind.

8. Wandelement (1) nach einem der vorangehenden Ansprüche 1 bis 7, wobei die Verstärkungsschicht(en) (3) aus Holz hergestellt ist bzw. sind.

9. Verfahren zum Herstellen eines flachen Wandelements (1) nach einem der vorangehenden Ansprüche 1 bis 8, **dadurch gekennzeichnet, daß** das Wandelement (1) wenigstens im wesentlichen hergestellt wird aus einer geraden Anzahl von Schichten aus Papier/Pappe, wobei jede Schicht wenigstens im wesentlichen hergestellt wird aus einer gewellten Unterschicht (4) und einer ebenen Unterschicht (5), die auf einer Seite derselben vorgesehen ist, welche Schichten aus Papier/Pappe über einen Klebstoff miteinander verbunden werden, der auf die Wellen (6) der gewellten Unterschichten (4) aufgetragen wird, wobei das Wandelement (1) mit einem harzartigen Material imprägniert wird, wobei wenigstens eine Verstärkungsschicht (3) mit einem größeren Elastizitätsmodul als die Schichten aus Papier/Pappe vorgesehen wird, welche Verstärkungsschicht (3) mit einer Schicht aus Papier/Pappe auf einer Seite des Wandelements (1) über einen Klebstoff verbunden ist, und wobei das Wandelement (1) spiegelsymmetrisch in Bezug auf eine zentrale Längsebene (7) des Wandelements (1) ist, wobei die wenigstens eine Verstärkungsschicht (3) einen Elastizitätsmodul von größer als oder gleich 50 GPA aufweist.

## Revendications

1. Panneau plat (1) de cloison formé au moins pratiquement d'un matériau à base de cellulose, dans lequel le panneau de cloison (1) est constitué au moins pratiquement de couches de papier-carton, chaque couche (4) étant constituée au moins pratiquement d'une sous-couche ondulée (5) et d'une sous-couche plate disposée d'un côté de la précédente, et les couches de papier-carton sont interconnectées par un adhésif, dans lequel le panneau de cloison (1) est imprégné, et dans lequel une couche de renforcement au moins (3) ayant un module d'élasticité supérieur à celui des couches de papier-carton est incorporée, et la couche de renforcement (3) est raccordée à une couche de papier carton d'un côté du panneau de cloison (1) par un adhésif, **caractérisé en ce que** le panneau de cloison (1) est imprégné d'un matériau résineux, et **en ce que** le panneau de cloison (1) est au moins pratiquement constitué d'un nombre pair de couches de papier-carton, et le panneau de cloison (1) présente une symétrie spéculaire par rapport à un plan longitudinal central (7) du panneau de cloison (1), la couche de renforcement au moins (3) ayant un module d'élasticité supérieur ou égal à 50 GPa.

2. Panneau de cloison (1) selon la revendication 1, dans lequel deux couches de renforcement (3) sont incorporées et sont raccordées par un adhésif à une couche de papier-carton de chaque côté du panneau de cloison (1).

3. Panneau de cloison (1) selon la revendication 1 ou 2, dans lequel la couche ou les couches de renforcement (3) comprennent un matériau fibreux,

4. Panneau de cloison (1) selon la revendication 3, dans lequel le matériau fibreux est constitué de fibres de verre, de fibres de carbone, de fibres minérales et/ou de fibres synthétiques.

5. Panneau de cloison (1) selon l'une quelconque des revendications précédentes 1 à 4, dans lequel la couche ou les couches de renforcement (3) comprennent une couche de matière plastique.

6. Panneau de cloison (1) selon l'une quelconque des revendications précédentes 1 à 5, dans lequel la couche ou les couches de renforcement (3) comprennent une couche de caoutchouc.

7. Panneau de cloison (1) selon l'une quelconque des revendications précédentes 1 à 6, dans lequel la couche ou les couches de renforcement (3) sont formées de métal.

8. Panneau de cloison (1) selon l'une quelconque des revendications précédentes 1 à 7, dans lequel la couche ou les couches de renforcement (3) sont formées de bois.

9. Procédé de fabrication d'un panneau plat de cloison (1) selon l'une quelconque des revendications précédentes, **caractérisé en ce que** le panneau de cloison (1) est formé au moins pratiquement d'un nombre pair de couches de papier-carton, chaque couche au moins étant pratiquement constituée d'une sous-couche ondulée (4) et d'une sous-couche plate (5) placée d'un côté de la précédente, les couches de papier-carton étant interconnectées par un adhésif appliqué aux ondulations (6) des sous-couches ondulées (4), **en ce que** le panneau de cloison (1) est imprégné d'un matériau résineux, **en ce qu'**au moins une couche de renforcement (3) ayant un module d'élasticité supérieur à celui des couches de papier-carbone est incorporé, cette couche de renforcement (3) étant raccordée à une couche de papier-carton d'un premier côté du panneau de cloison (1) par un adhésif, et **en ce que** le panneau de cloison (1) présente une symétrie spéculaire par rapport à un plan longitudinal central (7) du panneau de cloison (1), la couche de renforcement au moins (3) ayant un module d'élasticité supérieur ou égal à 50 GPa.
